

July 21, 1942.

C. H. HACK

2,290,554

METHOD OF FABRICATING REINFORCED MATERIAL

Filed June 27, 1940



INVENTOR  
Carl H. Hack  
BY Charles F. Langbehn  
John B. Henrich Jr.  
ATTORNEYS

## UNITED STATES PATENT OFFICE

2,290,554

## METHOD OF FABRICATING REINFORCED MATERIAL

Carl H. Hack, St. Albans, N. Y., assignor to National Lead Company, New York, N. Y., a corporation of New Jersey

Application June 27, 1940, Serial No. 342,713

1 Claim. (Cl. 29—189)

The present invention relates to the reinforcing of soft plastic materials, and particularly to the reinforcing of soft metals, the ductility of which permit their cold rolling.

For the sake of clarity my invention will be described with respect to the strengthening or reinforcement of sheet lead or alloys of lead.

Lead sheet is used for many purposes. Some of these uses are for flashings, roofing, and various architectural purposes, as well as for the lining of tanks and the like. Since lead is somewhat weak as a structural material, attempts have been made to either alloy the material in order to strengthen it, or to attach, support, line or otherwise mechanically stiffen the metal in some way or other. If the sheet is hung vertically by supporting attachments, it will often fail by creeping or buckling, due to its own weight, unless the design and the number of attachments or stresses are carefully planned, so as to relieve the strain on the lead sheet. Roofing will at times sag and elongate under the force of its weight, and this property of the metal is usually termed "crawling." The long time elongation or stretch of the metal under steady loads is due to the inherent plastic nature of the metal. Furthermore, lead has a considerable coefficient of expansion, and when it is subjected to periodic changes of temperature it tends to fail by buckling and subsequent cracking.

One of the objects of the present invention is to provide a stronger sheet lead or lead alloy which will overcome to a great degree the inherent tendency of lead to elongate, creep, buckle and crack. Other objects of my invention and novel features of construction will become apparent from the specification when considered together with the accompanying drawing, in which Fig. 1 is a perspective view of a suitable rolling apparatus and of my novel product before and after being rolled; Fig. 2 is a detailed view in cross section of my fabricated product; and Fig. 3 is a diagrammatic representation of the improved properties exhibited by my novel product.

As understood at the present time, stretching of a metal under tension may result in sudden failure in the space of a few minutes by reason of the imposition of a load too great for the metal to bear, but failure may also result by a very gradual process of elongation which can only be noted by careful measurements during the course of weeks or months. The first phenomenon is commonly tested for and denoted by what is known as the ultimate tensile strength, while the latter is called "creep." Lead sheet reinforced

according to the present invention has a tensile strength which is double, and in some cases more than double, the tensile strength of a similar product not reinforced. Moreover, my reinforced sheet lead displays a still more remarkable improvement as regards creep strength, being 7 or more times stronger than unreinforced sheet lead. This increase in strength is more apparent at elevated temperatures.

According to the practice of my invention a sheet of lead or of the common lead alloys, for example, antimonial lead, is reinforced with a wire mesh, wire cloth, or wire screening of such material as iron, tinned iron, galvanized iron, steel, stainless steel, monel, nickel, copper, brass, bronze or the like, which is suitably embedded in the sheet of lead, or, if desired, between two sheets of lead, it being understood that this latter product can be so fabricated as not to be subsequently thicker than the single lead sheet with the reinforcing means embedded therein. The thickness of the fabricated product will, of course, be dependent upon the use to which it is to be put.

With reference now to Figs. 1 and 2, in which similar numerals refer to similar parts, 1 represents a sheet of lead of any desired thickness which is placed flat on the bed 2 of a rolling mill of the type used in rolling lead. On top of this sheet of lead 1 is placed a wire-mesh screen 3.

With the passage space through the rolls 4 being approximately the same or a little less than the thickness of the sheet, the lead and the screen are simultaneously passed through the rolls. In order to insure the proper embedding of the wire-mesh

screen into the lead sheet, my invention contemplates re-passing the lead sheet through the rolls one or more times. However, in view of the fact that the amount of reduction of thickness of the lead sheet should be carefully controlled, since it is not desirable to force the wire to elongate, nor to elongate the lead so much that the ends thereof will lack the reinforcing properties of the wire screen, it is well to subject the lead sheet only to

such a number of rolling operations as may be sufficient properly to embed the wire mesh into the sheet. Generally speaking, twice passing the lead sheet through the rolls with a roll clearance space slightly smaller than the thickness of the sheet to be rolled is sufficient. Of course, the amount of the clearance space between the rolls will depend upon the hardness of the alloy to be rolled, and the size of the wire mesh used as a reinforcing agent. In the operation of my invention it is also desirable to have the lead flow over

the junctions of the wires in the mesh, thus locking the wires firmly into the lead sheet.

It is, of course, obvious that where plurality of rolling operations is desired, one or more additional sets of rolls arranged in a series, and each adjusted to a desired clearance space, may be employed. Moreover, not all of these rolls need be power-driven. Some may be rotated merely by the movement of the lead sheet therethrough, these rolls being known as "idlers."

To effect a more perfect bond between the wire mesh and the lead sheet, thus to insure the wire mesh being held in place regardless of the amount and degree of bending to which the reinforced sheet lead may be subjected, my invention primarily contemplates sweating the wires in the lead following the rolling operation. The procedure is as follows:

The reinforcing agent, for example, an iron wire screen, is first suitably coated with a soft solder. The lead sheet and the coated wire mesh are then passed together through the rolls in a manner similar to that described above. After rolling, the top side of the rolled lead sheet into which the wire mesh is embedded is coated with a suitable flux of zinc chloride, or the like, which may be applied by brushing, and placed in an oven for a short period of time, and heated at a temperature of about 230° C. until the solder-coating on the wire mesh is melted and the wire thus sweated firmly into the lead sheet. The temperature and time of the sweating operation may vary between wide limits, depending upon the alloy or the solder used. Usually, ten minutes are sufficient to accomplish the desired result. After being removed from the oven, the reinforced sheet lead is washed so as to remove the surplus zinc chloride therefrom.

The remarkably improved properties of the product reinforced according to my invention are vividly illustrated by the tables given below. Table I shows the ultimate tensile strength to failure on specimens of pure commercial lead sheets and antimonial lead sheets. These specimens were about 0.04" thick, and were pulled on the testing machine at a rate of about 0.5" per minute on a 2.0" test length. Table II illustrates the vastly increased resistance to creep imparted to sheets of lead and of antimonial lead when reinforced according to the present invention.

TABLE I

*Ultimate tensile strength of sheet lead and antimonial lead reinforced with iron wire mesh*

| Reinforcement                                                                        | Composition of sheet reinforced | Tensile strength expressed in lbs. per square inch |
|--------------------------------------------------------------------------------------|---------------------------------|----------------------------------------------------|
| None                                                                                 | Lead                            | 1,750                                              |
| 12 mesh x .011 diameter iron wire                                                    | Lead                            | 5,100                                              |
| 14 mesh x .017 diameter iron wire                                                    | Lead                            | 5,650                                              |
| 12 mesh x .011 diameter iron wire (wire mesh soldered or sweated in the metal sheet) | Lead                            | 5,500                                              |
| 14 mesh x .017 diameter iron wire (wire mesh soldered or sweated in the metal sheet) | Lead                            | 5,900                                              |
| None                                                                                 | 6% antimonial lead              | 4,100                                              |
| 14 mesh x .015 diameter iron wire                                                    | 6% antimonial lead              | 6,600                                              |
| 14 mesh x .015 diameter iron wire (wire mesh soldered or sweated in the metal sheet) | 6% antimonial lead              | 9,700                                              |

TABLE II  
*Creep strength—percent elongation under load*

|                   | Load per sq. inch                                                                                                                                                      | Time and percent creep           |                                         |                                          |                           |
|-------------------|------------------------------------------------------------------------------------------------------------------------------------------------------------------------|----------------------------------|-----------------------------------------|------------------------------------------|---------------------------|
|                   |                                                                                                                                                                        | 2 weeks                          | 4 weeks                                 | 8 weeks                                  |                           |
| <i>Specimen A</i> |                                                                                                                                                                        |                                  |                                         |                                          |                           |
| 10                | Lead sheet having an overall thickness of .040"—not reinforced                                                                                                         | 200<br>400<br>600<br>800         | 0.03<br>.43<br>2.60<br>Broke in one day | 0.07<br>.77<br>.30                       | 0.10<br>1.33<br>10.7      |
| <i>Specimen B</i> |                                                                                                                                                                        |                                  |                                         |                                          |                           |
| 15                | Lead sheet having an overall thickness of .040" reinforced with 14 mesh wire of .017" diameter                                                                         | 1,250<br>1,750<br>2,250<br>3,000 | 0.00<br>.00<br>.00<br>.10               | 0.00<br>.03<br>.03<br>.17                | 0.00<br>.03<br>.07<br>.23 |
| <i>Specimen C</i> |                                                                                                                                                                        |                                  |                                         |                                          |                           |
| 20                | Lead sheet having an overall thickness of .046" reinforced with 14 mesh wire of .017" diameter which has been sweated or soldered in the lead sheet                    | 1,250<br>1,750<br>2,250<br>3,000 | 0.00<br>.03<br>.00<br>.03               | 0.00<br>.03<br>.00<br>.07                | 0.00<br>.07<br>.03<br>.10 |
| <i>Specimen D</i> |                                                                                                                                                                        |                                  |                                         |                                          |                           |
| 25                | 7% antimonial lead sheet having an overall thickness of .050"—not reinforced                                                                                           | 400<br>600<br>800<br>1,000       | 0.07<br>.90<br>4.83<br>17.7             | 0.13<br>1.70<br>10.1<br>Broke in 20 days | 0.27<br>3.17<br>21.9      |
| <i>Specimen E</i> |                                                                                                                                                                        |                                  |                                         |                                          |                           |
| 30                | 6% antimonial lead having an overall thickness of .043" reinforced with 14 mesh wire of .015" diameter                                                                 | 1,250<br>1,750<br>2,250<br>3,000 | 0.00<br>.00<br>.10<br>.13               | 0.00<br>.00<br>.10<br>.20                | 0.00<br>.00<br>.17<br>.30 |
| <i>Specimen F</i> |                                                                                                                                                                        |                                  |                                         |                                          |                           |
| 35                | 6% antimonial lead having an overall thickness of .045" reinforced with 14 mesh wire of .015" diameter which has been sweated or soldered in the antimonial lead sheet | 1,250<br>1,750<br>2,250<br>3,000 | 0.00<br>.00<br>.03<br>.10               | 0.00<br>.00<br>.03<br>.23                | 0.00<br>.00<br>.07<br>.37 |

To more clearly illustrate the data embodied in Table II, reference is made to Fig. III, which graphically sets forth the contents of this table. This graphic illustration is self-explanatory, and no further elaboration is necessary.

It is to be understood that the foregoing description of my invention has been given merely for illustrative purposes, and no undue limitations should be deduced therefrom. Thus, it is to be understood that the scope of my invention is sufficiently broad to embrace the reinforcing of lead or lead alloy sheets with wire mesh on both top and bottom sides. Furthermore, the reinforcement may be accomplished by placing wire mesh between two lead or lead alloy sheets, and then rolling the same, as hereinabove described.

Also, it is to be understood that the reinforcement of the sheet may be accomplished by means other than rolling, such as, for instance, placing the lead sheet, together with the wire mesh, in a press or by extruding lead ribbon together with the wire mesh in a manner similar to the method of extruding cable sheathing around cable.

I claim:

A process for making a reinforced lead or lead alloy sheet which comprises coating a wire mesh screen with a soft solder, placing the treated wire mesh screen on a metal sheet, simultaneously subjecting the said metal sheet and wire mesh screen to at least one cold-rolling operation, thereby to embed the wire mesh screen into the metal sheet, coating with a suitable flux the embedded wire mesh screen surface of the metal sheet, heating the same until the solder coating is melted and washing away the surplus flux.

CARL H. HACK.